# EUROPEAN PATENT SPECIFICATION

(11) **EP 2 327 831 B1**
(45) Date of publication and mention of the grant of the patent: **22.01.2014**
(21) Application number: 09812813.5
(22) Date of filing: 01.06.2009
(51) Int. Cl.: D06M 11/63, D06M 11/00, D06M 11/38, D06M 11/50, D06M 101/28

(54) **A CROSS-LINKED ACRYLATE FIBER AND A METHOD FOR MANUFACTURING IT**
VERNETZTE FASERN AUF ACRYLATBASIS UND IHRE HERSTELLUNG
FIBRES RÉTICULÉES À BASE D'ACRYLATE ET LEUR PRODUCTION

(30) Priority: 10.09.2008 JP 2008231582
(43) Date of publication of application: 01.06.2011
(73) Proprietor: JAPAN EXLAN COMPANY LIMITED, Osaka-shi Osaka 530-0004 (JP)
(72) Inventor: YAMAUCHI, Takao, Okayama-shi Okayama 704-8510 (JP); TANAKA, Koji, Okayama-shi Okayama 704-8510 (JP)
(74) Representative: Patentanwälte Ruff, Wilhelm, Beier, Dauster & Partner
(86) International application number: PCT/JP2009/002428
(87) International publication number: WO 2010/029664

(56) References cited:
- WO-A1-2009/057235
- JP-A- 2 210 062
- JP-A- 9 158 040
- JP-A- 2002 294 556
- JP-A- 2003 278 079
- JP-A- 2006 070 421
- DATABASE WPI Week 200446 Thomson Scientific, London, GB; AN 2004-483177 XP002680391, & JP 2004 149989 A (TEIJIN LTD) 27 May 2004 (2004-05-27)
- DATABASE WPI Week 197744 Thomson Scientific, London, GB; AN 1977-78105Y XP002680392, & JP 50 126996 A (MITSUBISHI RAYON CO LTD) 6 October 1975 (1975-10-06)

## Description

### Technical Field

The present invention relates to a cross-linked acrylate fiber and to a method for manufacturing the same. More particularly, it relates to a cross-linked acrylate fiber having a color which induces no unusual sense in the appearance when used in the industrial material field together with other fibers for industrial materials.

### Background Art

Cross-linked acrylate fiber has been known to have various functions such as absorption/desorption property for moisture, moisture-absorption exothermic property, deodorant property, antibacterial property and flame-resisting property and is a fiber which is expected to be developed to various fields. However, since the fiber is in pink color and it further turns dark upon a post-treatment and with elapse of time, there is a problem that development of its use has been limited. For such a problem, many investigations have been carried out for a purpose of development to the field of clothing.

For example, investigations for improving the whiteness are done in Patent Documents 1 to 3 and a cross-linked acrylate fiber having the whiteness in a practically acceptable level is achieved. In Patent Document 4, there is disclosed a cross-linked acrylate fiber in black color prepared from black-doped acrylic fiber as a material. Further, in Patent Documents 5 and 6, investigations are conducted for making cross-linked acrylate fiber into various colors by dyeing. However, with regard to dyeing, further investigations are still necessary for achieving the practically sufficient product in view of hue stability, uneven dyeing, fastness in dyeing, etc.

As mentioned above, although various investigations have been done for the color of cross-linked acrylate fiber in the prior art for a purpose of development to the filed of clothing, only limited colors in a practical level have been provided.

On the other hand, restriction in the color of cross-linked acrylate fiber is not negligible in the field of industrial materials as well. In the industrial material field, there are many cases where various types of fibers for industrial materials are mixed and made into products and, with regard to the color of the fibers for industrial materials, that similar to golden color is abundant. Therefore, when the cross-linked acrylate fiber with the above color is used together, unusual sense is resulted in the appearance of the product. Although white color has less unusual sense as compared with pink and black colors, many steps are needed for enhancing the whiteness whereby cost therefor is high and that is hardly acceptable. As such, although the conventional cross-linked acrylate fibers have various functions as mentioned above, the current state is that they are hardly developed to the field of industrial materials.

It has been also known that the cross-linked acrylate fiber has a flame resisting property as mentioned above and, particularly when carboxyl group in the fiber is made into a magnesium salt type, the resulting cross-linked acrylate fiber has a very high flame resisting property which is not found in the common organic fibers (Patent Document 7). Such a cross-linked acrylate fiber of a magnesium salt type also has a characteristic of slow moisture absorption/desorption property or, in other words, the speed of absorption and desorption of moisture is slow (Patent Document 8). Therefore, a continued generation of heat by means of absorption of moisture is possible and that is particularly useful in the field of clothing.

However, the above fact shows that, in the prior art, high flame resisting property and high moisture absorption/desorption speed are incompatible in the cross-linked acrylate fiber of a magnesium salt type and development to the use where such a characteristic is demanded is not possible.

### Prior Art Documents

### Patent Documents

Patent Document 1: Japanese Patent Application Laid-Open (JP-A) No. 158040/97
Patent Document 2: Japanese Patent Application Laid-Open (JP-A) No. 2000-303353
Patent Document 3: Japanese Patent Application Laid-Open (JP-A) No. 2002-294556
Patent Document 4: Japanese Patent Application Laid-Open (JP-A) No. 2003-89971
Patent Document 5: Japanese Patent Application Laid-Open (JP-A) No. 2003-278079
Patent Document 6: Japanese Patent Application Laid-Open (JP-A) No. 2006-70421
Patent Document 7: WO 2006/027911
Patent Document 8: WO 2006/027910

A method for producing an acrylic-group fiber having high moisture absorption property is known from JP 2004/149989 A. The method is based on a) cross-linking process, b) hydrolyzing process and c) oxidization treatment and alkali treatment.

### Summary of the Invention

### Problem that the Invention is to Solve

An object of the present invention is to provide a cross-linked acrylate fiber having the color causing no unusual sense in the appearance even when used together with other fibers for industrial materials in the field of industrial materials which has not been provided in the prior art and also being advantageous in terms of the cost. Another object of the present invention is to provide a cross-linked acrylate fiber having both of the high flame resisting property and the high speed of moisture absorption/desorption.

### Means for Solving the Problem

The above-mentioned objects of the present invention can be achieved by the following means. Thus:
[1] A cross-linked acrylate fiber having a color where L* is 60 to 75, a* is 5.0 to 14.5 and b* is 23.0 to 30.0 in accordance with the expression method stipulated by JIS-Z-8729.
[2] The cross-linked acrylate fiber according to [1], wherein the treatments of (a) treatment for introduction of cross-linking by a hydrazine compound, (b) treatment by a peroxide and (c) hydrolyzing treatment using an alkaline metal compound are applied to an acrylonitrile fiber in the order of (a), (b) and (c) or in such an order that, after (a) is applied, (b) and (c) are then applied together.
[3] The cross-linked acrylate fiber according to [1] or [2], wherein the counter ion (s) for at least a part of carboxyl groups in the cross-linked acrylate fiber are/is magnesium and/or zinc ion.
[4] The cross-linked acrylate fiber according to [3], wherein the counter ion for at least a part of carboxyl groups in the cross-linked acrylate fiber is magnesium ion, the limit oxygen index is 30 to 50 and the saturated moisture absorption rate is 20 to 60% by weight.
[5] A method for the manufacture of a cross-linked acrylate fiber, characterized in that, the treatments of (a) treatment for introduction of cross-linking by a hydrazine compound, (b) treatment by a peroxide and (c) hydrolyzing treatment using an alkaline metal compound are applied to an acrylonitrile fiber in the order of (a), (b) and (c).
[6] A method for the manufacture of a cross-linked acrylate fiber, characterized in that, the treatments of (a) treatment for introduction of cross-linking by a hydrazine compound, (b) treatment by a peroxide and (c) hydrolyzing treatment using an alkaline metal compound are applied to an acrylonitrile fiber in such an order that, after (a) is applied, (b) and (c) are then applied together.

### Advantages of the Invention

Since the color of the cross-linked acrylate fiber of the present invention is similar to golden color, it does not cause unusual sense even when mixed with a fiber for industrial materials and, further since the manufacturing steps are fewer and the cost therefor can be suppressed, the fiber can be advantageously used in the field of industrial materials. In addition, in the cross-linked acrylate fiber of the present invention, a high moisture absorption/desorption speed can be achieved and both of the high flame resisting property and the high moisture absorption/desorption speed which could not be achieved in the conventional cross-linked acrylate fiber are available whereby it is now possible to develop to the uses where such characteristics have been demanded.

### Brief Descriptions of Drawings

Fig. 1 shows moisture absorption curves of the cross-linked acrylate fibers of Examples 1 and 2 and Comparative Example 1 and 2.

### Best Mode for Carrying Out the Invention

The present invention will now be illustrated in detail as hereunder.

Since the color of the cross-linked acrylate fiber of the present invention is similar to golden color which has never been achieved in the conventional cross-linked acrylate fiber, it causes no unusual sense even when mixed with a fiber for industrial materials. To be more specific, it is the color where L* is 60 to 75, a* is 5.0 to 14.5 and b* is 23.0 to 30.0 in accordance with the indication method stipulated by JIS-Z-8729 and the color where L* is 65 to 75, a* is 7.0 to 13.0 and b* is 23.5 to 27.0 is preferred.

The cross-linked acrylate fiber of the present invention as such can be manufactured according to such a manner that each of the treatments of (a) treatment for introduction of cross-linking by a hydrazine compound, (b) treatment by a peroxide and (c) hydrolyzing treatment using an alkaline metal compound are applied to an acrylonitrile fiber in the order of (a), (b) and (c) or in such an order that, after (a) is applied, (b) and (c) are then applied together.

The acrylonitrile fiber adopted in the present invention is manufactured from an acrylonitrile polymer by a known method and, as to the composition of said polymer, amount of acrylonitrile is preferably not less than 40% by weight, more preferably not less than 50% by weight and, still more preferably, not less than 80% by weight. As will be mentioned later, a hydrazine compound is made to react with nitrile group of the acrylonitrile polymer forming the acrylonitrile fiber to introduce a cross-linking structure into the fiber of the present invention. Cross-linking structure greatly affects the properties of the fiber and, when the copolymerizing composition of acrylonitrile is too small, the cross-linking structure naturally becomes small and there is a possibility that the properties of the fiber become insufficient but, when the copolymerizing composition of the acrylonitrile is made within the above range, a good result is apt to be achieved.

Examples of the copolymerizing component other than acrylonitrile in the acrylonitrile polymer include a sulfonic acid-containing monomer such as methallylsulfonic acid or p-styrenesulfonic acid and a salt thereof; a carboxylic acid-containing monomer such as (meth) acrylic acid or itaconic acid and a salt thereof; and a monomer such as styrene, vinyl acetate, (meth)acrylate or (meth)acrylamide and there is no particular limitation therefor so far as it is a monomer being able to be copolymerized with acrylonitrile.

The form of the acrylonitrile fiber adopted by the present invention may be any of the forms of short fiber, tow, yarn, knitted/woven fabric, nonwoven fabric, etc. and even an intermediate during the manufacture, waste fiber, etc. may be adopted as well.

When the acrylonitrile fiber is treated with a solution containing a hydrazine compound in the treatment (a), hydrazine reacts with the nitrile group of the acrylonitrile fiber whereupon a cross-linking structure is formed in the fiber. Examples of the hydrazine compound include hydrazine hydrate, hydrazine hydrochloride, hydrazine sulfate, neutral hydrazine sulfate and hydrazine carbonate. An example of the treating condition is that the above acrylonitrile fiber is dipped in an aqueous solution to which the above hydrazine compound is added so as to make the hydrazine concentration 3 to 40% by weight followed by treating at 50 to 120°C for not longer than 5 hours.

In the treatment (b), the fiber prepared by subjecting to the treatment (a) is treated with a solution containing a peroxide. As a result of such a treatment, color of the finally prepared cross-linked acrylate fiber can be made similar to golden color. Examples of the peroxide used for the treatment include hydrogen peroxide, ammonium persulfate and potassium persulfate. An example of the treating condition is that the fiber is dipped in an aqueous solution where the peroxide concentration is 1 to 15% by weight or, preferably, 3 to 8% by weight and treated at 50 to 120°C for 0.5 to 20 hour (s) . It is preferred that, before the treatment, the fiber is well washed with water so that the chemicals remained in the treatment (a) are removed as much as possible.

The treatment (c) is a hydrolyzing treatment using an alkaline metal compound. As a result of the treatment, nitrile group and amide group existing in the fiber are hydrolyzed to form carboxyl group. The carboxylic group is an important factor for expressing the characteristic such as moisture absorption/desorption property, moisture-absorption exothermic property or deodorizing property in the cross-linked acrylate fiber and it is desirable to form 1 to 12 mmol/g, preferably 3 to 10 mmol/g or, more preferably 3 to 8 mmol/g of carboxyl group in terms of the total carboxyl group amount. Amount of the carboxyl group formed thereby may be adjusted by the treating condition. Incidentally, amide group is produced from a part of nitrile group during the treatment (a).

Examples of the alkaline metal compound used in the treatment (c) include alkali metal hydroxide such as sodium hydroxide or potassium hydroxide; and alkali metal carbonate such as sodium carbonate. An example of the treating condition is that the fiber is dipped in an aqueous solution where the alkaline metal compound is 1 to 10% by weight or, preferably, 1 to 5% by weight followed by treating at 50 to 120°C for 1 to 10 hour(s). Counter ion for the carboxyl group formed thereby is a metal ion corresponding to the alkaline metal compound used therefor.

It is also possible that the above treatments (b) and (c) are applied at the same time. In that case, the fiber which was prepared by the treatment (a) may be treated by dipping in a solution containing both of the above-mentioned peroxide and the alkaline metal compound.

As mentioned above, the cross-linked acrylate fiber of the present invention can be prepared by applying the treatments (a), (b) and (c) to the acrylonitrile fiber and it is also possible that the carboxyl group in the fiber is made into a desired salt-type carboxyl group or H-type carboxyl group by subjecting to an ion-exchange treatment using metal salt such as nitrate, sulfate or hydrochloride, to an acid treatment using nitric acid, sulfuric acid, hydrochloric acid, formic acid, etc. or to a pH-adjusting treatment using an alkaline metal compound, etc. or that a salt-type carboxylic group of a different type is made to contain therein so that the characteristic such as moisture absorption/desorption property, exothermic property upon moisture absorption, deodorizing property, antibacterial property or flame resisting property can be adjusted.

With regard to the metal which constitutes the salt-type carboxylic group, one or more member(s) may be selected from alkali metal such as lithium, sodium or potassium, alkali earth metal such as magnesium or calcium and other metal such as manganese, copper, zinc or silver depending upon the required characteristic.

With regard to the moisture absorption/desorption property, a salt-type carboxyl group such as sodium, potassium, magnesium or calcium is suitable and, when the cross-linked acrylate fiber of the present invention is compared with the conventional cross-linked acrylate fiber to which no peroxide treatment is applied, the cross-linked acrylate fiber of the present invention has a characteristic that the moisture absorption speed can be made relatively high whereby far better moisture absorption/desorption property can be achieved even in such a case where, in both fibers, the metals for the salt-type carboxyl group are same and the saturated moisture absorption rates are homologous as well.

For a purpose of enhancing the flame resisting property which is important in the field of industrial materials, it is desirable to select magnesium salt-type carboxyl group or zinc salt-type carboxyl group as the salt-type carboxyl group. With regard to the amount of the salt-type carboxyl group as such, it is preferably not less than 2 mmol/g in terms of an absolute amount and not less than 50% to the total carboxyl group amount, more preferably not less than not less than 2 mmol/g in terms of an absolute amount and not less than 60% to the total carboxyl group amount or not less than not less than 3 mmol/g in terms of an absolute amount and not less than 50% to the total carboxyl group amount and, most preferably, not less than not less than 3 mmol/g in terms of an absolute amount and not less than 60% to the total carboxyl group amount. A method for making into such a salt-type carboxyl group will be illustrated as follows taking a magnesium salt-type carboxyl group as an example.

Thus, in preparing a cross-linked acrylate fiber having a magnesium salt-type carboxyl group, it can be manufactured by dipping the fiber after the treatment (c) into an aqueous solution containing magnesium ion such as an aqueous solution of magnesium nitrate. If the amount of the magnesium salt-type carboxylic group is to be more precisely controlled, the following method may be adopted.

Firstly, the fiber after the treatment (c) is dipped in an aqueous acid solution such as nitric acid so that the whole carboxyl group in the fiber is made into an H-type carboxyl group. After that, the resulting fiber is dipped in an alkaline aqueous solution containing sodium ion such as an aqueous solution of sodium hydroxide so that the H-type carboxyl group is made into a sodium salt-type carboxyl group. When the pH is adjusted at that time, the amount of the carboxyl group to be converted to the sodium salt type can be modified.

After that, the above is dipped in an aqueous solution containing magnesium such as an aqueous solution of magnesium nitrate to convert to a magnesium salt-type carboxyl group. Here, the group which can be converted to magnesium salt-type carboxyl group is sodium salt-type carboxyl group only and an H-type carboxyl group is hardly converted to a magnesium salt-type carboxyl group. Thus, by means of controlling the amount of the sodium salt-type carboxyl group by adjusting the pH, it is possible to control the amount of the magnesium salt-type carboxyl group. Further, since the conversion of the sodium salt-type carboxyl group into the magnesium salt-type one is a reversible reaction, it is also possible that chemical equilibrium is shifted by the amount of magnesium ion in a solution containing magnesium ion so that the amount of magnesium salt-type carboxyl group is controlled.

The magnesium salt-type cross-linked acrylate fiber of the present invention prepared as such has the identical flame resisting property to that of the conventionally known magnesium salt-type cross-linked acrylate fiber and a limit oxygen index of 30 to 50 or, preferably, 35 to 50 can be achieved. Further, said fiber has a saturated moisture absorption rate of 20 to 60% by weight or, preferably, 30 to 60% by weight and, with regard to the moisture absorption speed, a moisture absorption rate during five minutes under the atmosphere of 20°C and 65% RH is higher to an extent of two fold or more as compared with the conventional magnesium salt-type cross-linked acrylate fiber which has the same degree of saturated moisture absorption rate as the magnesium salt-type cross-linked acrylate fiber of the present invention, whereby the coexistence of high flame resisting property and high moisture absorption speed which has not been available in the past is now able to be achieved.

The cross-linked acrylate fiber of a zinc salt type can also be prepared by the same method as in the case of the cross-linked acrylate fiber of a magnesium salt type mentioned above. In that case, an aqueous solution containing zinc ion such as aqueous solution of zinc chloride, zinc nitrate or zinc sulfate may be used in place of the above-mentioned aqueous solution containing magnesium ion such as magnesium nitrate.

Although the reason why a cross-linked acrylate fiber in a color similar to golden color can be prepared in the present invention is not clear, it is likely that changes in a tetrazine ring structure take place by the treatment with a peroxide in the present invention since it has been believed that the pink color of the conventional cross-linked acrylate fiber is due to a tetrazine ring structure formed by the treatment for introduction of cross-linking by a hydrazine compound.

### Examples

The present invention will now be more specifically illustrated by way of the following Examples although the present invention is not limited by the following Examples. The terms "part(s)" and "%" in the Examples are those by weight unless otherwise mentioned. Firstly, method for evaluation of each characteristic and method for representation of the evaluation result will be explained.

### [Amount of total carboxyl group]

A well-dried sample (about 1 g) was precisely weighted (W1 [g]), 200 ml of 1 mol/l aqueous solution of hydrochloric acid was added thereto and the mixture was allowed to stand for 30 minutes, filtered through a glass filter and washed with water after addition of water. The treatment was repeated for three times and well washed with water until pH of the filtrate became 5 or higher. After that, this sample was placed in 200 ml of water, the mixture was adjusted to pH 2 by addition of 1 mol/l aqueous solution of hydrochloric acid thereto and a titration curve is determined by a common method using a 0. 1 mol/l aqueous solution of sodium hydroxide. From said titration curve, amount (V1[ml]) of the aqueous solution of sodium hydroxide consumed by carboxyl group is determined and an amount of total carboxyl group is calculated by the following formula. $Amount of total carboxyl group \left(mmol/g\right) = \left(0.1*V⁢1\right) / W ⁢ 1$

### [Amount of salt-type carboxyl group]

A well-dried sample is precisely weighed, subjected to an acid decomposition by a common method using a mixed solution of concentrated sulfuric acid and concentrated nitric acid and metal contained in a form of a salt of carboxyl group is quantified by an atomic absorption spectroscopy by a common method and divided by atomic weight of said metal to calculate an amount of salt-type carboxyl group.

### [Saturated moisture absorption rate]

A sample (about 5.0 g) is dried using a hot-air drier at 105°C for 16 hours to measure its weight (W2[g]). After that, the said sample is placed in a thermo-hygrostat kept at 20°C temperature and 65% relative humidity for 24 hours. Weight of the sample moisturized as such is measured (W3[g]). From the above measurement results, a saturated moisture absorption rate is calculated by the following formula. $Saturated moisture absorption rate \left(%\right) = \left[\left(W⁢3-W⁢2\right)/W⁢2\right] * 100$

### [Moisture absorption curve]

A sample (about 2.5 g) was dried at 105°C for 16 hours using a hot-air drier to measure the weight (W4 [g]). Then the sample was quickly placed in a cylindrical mesh basket (diameter: 7.5 cm; height: 9.8 cm) without pushing so as to make airy and immediately placed in a thermo-hygrostat (20°C/65%RH) without taking out from the basket. The stage of placing into said thermo-hygrostat was adopted as the starting point for absorption of moisture and weights of the moistened sample of 5, 10, 20 and 30 minutes thereafter were measured (W5 [g]). From the above measured result, moisture absorption rate for each measured stage was calculated according to the following formula and a moisture absorption curve was determined. $Moisture absorption rate \left(%\right) = \left[\left(W⁢5-W⁢4\right)/W⁢4\right] * 100$

### [Limiting oxygen index (LOI)]

A nonwoven fabric where the basis weight was 180 g/m² was prepared using a sample fiber and said nonwoven fabric was subjected to the measurement of LOI in accordance with the measuring method stipulated by JIS-K-7201-2. When the resulting value was high, it means that the flame resisting property was also high.

### [Fiber Color]

Color of the sample where the fiber was opened was measured for three times using a colorimeter CR 300 (illuminant: D65) manufactured by Minolta and the mean value of each of L*, a* and b* according to the indication method according to JIS-Z-8729 was determined.

### [Example 1]

A dope solution for spinning was prepared by dissolving an acrylonitrile polymer comprising 90% of acrylonitrile and 10% of methyl acrylate in a 48% aqueous solution of sodium thiocyanate. It was subjected to spinning, water-washing, stretching, crimping and heating treatments according to the conventional means to give a material fiber of 0.9 dtex and 70 mm. The material fiber was dipped in a 15% aqueous solution of hydrazine hydrate in a bath ratio of 1:10 and treated under the condition of 120°C for 1 hour. The resulting fiber was washed with water, dipped in a 4% aqueous solution of ammonium persulfate in a bath ratio of 1:10 and subjected to a peroxide treatment under the condition of 100°C for 1 hour. After that, the resulting fiber was dipped in a 5% aqueous solution of sodium hydroxide in a bath ratio of 1:10, hydrolyzed under the condition of 110°C for 1 hour and washed with water to give a cross-linked acrylate fiber of a sodium salt type. Results of evaluation for the characteristic of the resulting fiber are shown in Table 1 and Fig. 1.

### [Comparative Example 1]

The same operation as in Example 1 was carried out except that no peroxide treatment was conducted to give a cross-linked acrylate fiber of a sodium salt type. Results of evaluation for the characteristic of the resulting fiber are shown in Table 1 and Fig. 1.

### [Example 2]

The cross-linked acrylate fiber prepared in Example 1 was treated with a 1 mol/l aqueous solution of nitric acid so that the carboxyl group was converted into H type, washed with water, adjusted to pH 12 with 1 mol/l sodium hydroxide and washed with water to give a fiber having a sodium salt-type carboxyl group. The resulting fiber was dipped in an aqueous solution containing magnesium nitrate in an amount of 1.2 times equivalent of the carboxyl group amount of said fiber to subject to a converting treatment to a magnesium salt type under the condition of 50°C for 1 hour followed by washing with water whereupon a cross-linked acrylate fiber of a magnesium salt type was prepared. Results of evaluation for the characteristic of the resulting fiber are shown in Table 1 and Fig. 1.

### [Comparative Example 2]

The same operation as in Example 2 was conducted except that the cross-linked acrylate fiber prepared in Comparative Example 1 was used in place of the cross-linked acrylate fiber prepared in Example 1 to give a cross-linked acrylate fiber of a magnesium salt type. Results of evaluation for the characteristic of the resulting fiber are shown in Table 1 and Fig. 1.

### [Example 3]

The same operation as in Example 1 was conducted except that the peroxide treatment was done using a 3% aqueous hydrogen peroxide to give a cross-linked acrylate fiber of a sodium salt type. Results of evaluation for the characteristic of the resulting fiber are shown in Table 1.

### [Example 4]

The material fiber used in Example 1 was dipped in a 15% aqueous solution of hydrazine hydrate in a bath ratio of 1:10 and treated under the condition of 120°C for 1 hour followed by washing with water. The resulting fiber was dipped in an aqueous solution containing 4% of ammonium persulfate and 5% of sodium hydroxide in a bath ratio of 1:10 and subjected to a simultaneous treatment comprising a treatment with peroxide and a hydrolyzing treatment followed by washing with water to give a cross-linked acrylate fiber of a sodium salt type. Results of evaluation for the characteristic of the resulting fiber are shown in Table 1.

### [Example 5]

A dope solution for spinning was prepared by dissolving an acrylonitrile polymer comprising 88% of acrylonitrile and 12% of vinyl acetate in a 48% aqueous solution of sodium thiocyanate. It was subjected to spinning, water-washing, stretching, crimping and heating treatments according to the conventional means to give a material fiber of 0.9 dtex and 70 mm. The material fiber was dipped in a 15% aqueous solution of hydrazine hydrate in a bath ratio of 1:10 and treated under the condition of 120°C for 1.5 hours. The resulting fiber was washed with water, dipped in a 3% aqueous solution of potassium persulfate in a bath ratio of 1:10 and subjected to a peroxide treatment under the condition of 60°C for 30 minutes. After that, the resulting fiber was dipped in a 5% aqueous solution of sodium hydroxide in a bath ratio of 1:10, hydrolyzed under the condition of 110°C for 1 hour and washed with water to give a cross-linked acrylate fiber of a sodium salt type. Then, the said fiber was treated with a 1 mol/l aqueous solution of nitric acid so that the carboxyl group was converted into H type, washed with water, adjusted to pH 12 with 1 mol/l sodium hydroxide and washed with water to give a fiber having a sodium salt-type carboxyl group. The resulting fiber was dipped in an aqueous solution containing zinc sulfate in an amount of 1.3 times equivalent of the carboxyl group amount of said fiber to subject to a converting treatment to a zinc salt type under the condition of 50°C for 1 hour followed by washing with water whereupon a cross-linked acrylate fiber of a zinc salt type was prepared. Results of evaluation for the characteristic of the resulting fiber are shown in Table 1.

### [Example 6]

The cross-linked acrylate fiber prepared in Example 1 was treated with a 1 mol/l aqueous solution of nitric acid so that the carboxyl group was converted into H type, washed with water, adjusted to pH 12 with 1 mol/l sodium hydroxide and washed with water to give a fiber having a sodium salt carboxyl group. The resulting fiber was dipped in an aqueous solution containing magnesium nitrate in an amount of 1.6 times equivalent of the carboxyl group amount of said fiber to subject to a converting treatment to a magnesium salt type under the condition of 50°C for 1 hour followed by washing with water whereupon a cross-linked acrylate fiber of a magnesium salt type was prepared. Results of evaluation for the characteristic of the resulting fiber are shown in Table 1.

**[Table 1]**

| | Example 1 | Comparative Example 1 | Example 2 | Comparative Example 2 | Example 3 | Example 4 | Example 5 | Example 6 |
|---|---|---|---|---|---|---|---|---|
| Amount of total carboxyl group [mmol/g] | 5.5 | 6.5 | 5.5 | 6.5 | 5.3 | 5.0 | 5.2 | 5.5 |
| Salt type | Sodium | Sodium | Magnesium | Magnesium | Sodium | Sodium | Zinc | Magnesium |
| Amount of salt-type carboxylic group [mmol/g] | 3.9 | 4.5 | 3.5 | 4.1 | 3.7 | 3.6 | 3.2 | 4.6 |
| Moisture absorption rate [%] | 38 | 41 | 35 | 41 | 36 | 35 | 23 | 38 |
| LOI | 23 | 24 | 38 | 39 | 23 | 22 | 37 | 44 |
| Hue | golden color | pink color | golden color | pink color | golden color | golden color | golden color | golden color |
| L* | 69.3 | 66.6 | 68.7 | 65.6 | 69.1 | 68.2 | 67.8 | 68.3 |
| a* | 10.0 | 34.2 | 11.9 | 35.8 | 8.9 | 7.5 | 11.1 | 12.1 |
| b* | 26.5 | 8.9 | 24.7 | 8.8 | 27.3 | 26.6 | 24.8 | 24.5 |

As will be apparent from Table 1, the cross-linked acrylate fibers of Comparative Examples 1 and 2 have a pink color while the cross-linked acrylate fibers of Examples 1 to 6 being subjected to a peroxide treatment have a golden color. Further, as will be apparent from Fig. 1, although the cross-linked acrylate fibers of Examples 1 and 2 contain less amount of salt-type carboxyl group as compared with the cross-linked acrylate fibers of Comparative Examples 1 and 2, respectively, the moisture absorption rate after 5 minutes from the initiation of moisture absorption is 28% in Example 1 while that in Comparative Example 1 is 20% in the case of a sodium salt type and, in the case of a magnesium salt type, that is 6% in Example 2 while that in Comparative Example 2 is 2%. Thus, an increase in the moisture absorption speed is significant in a magnesium salt type.

## Claims

1. A cross-linked acrylate fiber having a color where L* is 60 to 75, a* is 5.0 to 14.5 and b* is 23.0 to 30.0 in accordance with the expression method stipulated by JIS-Z-8729.

2. The cross-linked acrylate fiber according to claim 1, wherein the treatments of (a) treatment for introduction of cross-linking by a hydrazine compound, (b) treatment by a peroxide and (c) hydrolyzing treatment using an alkaline metal compound are applied to an acrylonitrile fiber in the order of (a), (b) and (c) or in such an order that, after (a) is applied, (b) and (c) are then applied together.

3. The cross-linked acrylate fiber according to claim 1 or 2, wherein the counter ion (s) for at least a part of carboxyl groups in the cross-linked acrylate fiber are/is magnesium and/or zinc ion.

4. The cross-linked acrylate fiber according to claim 3, wherein the counter ion for at least a part of carboxyl groups in the cross-linked acrylate fiber is magnesium ion, the limit oxygen index is 30 to 50 and the saturated moisture absorption rate is 20 to 60% by weight.

5. A method for the manufacture of a cross-linked acrylate fiber, **characterized in that**, the treatments of (a) treatment for introduction of cross-linking by a hydrazine compound, (b) treatment by a peroxide and (c) hydrolyzing treatment using an alkaline metal compound are applied to an acrylonitrile fiber in the order of (a), (b) and (c).

6. A method for the manufacture of a cross-linked acrylate fiber, **characterized in that**, the treatments of (a) treatment for introduction of cross-linking by a hydrazine compound, (b) treatment by a peroxide and (c) hydrolyzing treatment using an alkaline metal compound are applied to an acrylonitrile fiber in such an order that, after (a) is applied, (b) and (c) are then applied together.

## Patentansprüche

1. Vernetzte Acrylatfaser mit einer Farbe, bei der, gemessen nach dem Standard-verfahren JIS-Z-8729, L* von 60 bis 75 beträgt, a* von 5,0 bis 14,5 beträgt und b* von 23,0 bis 30,0 beträgt.

2. Vernetzte Acrylatfaser nach Anspruch 1, bei der die Behandlungen (a) Behandlung zum Einbringen einer Vernetzung mit einer Hydrazinverbindung, (b) Behandlung mit einem Peroxid und (c) Hydrolysebehandlung mit einer Alkalimetallverbindung an einer Acrylnitrilfaser in der Abfolge (a), (b) und (c) oder in einer Abfolge derart vorgenommen werden, dass nachdem (a) erfolgt ist, (b) und (c) dann gemeinsam vorgenommen werden.

3. Vernetzte Acrylatfaser nach Anspruch 1 oder 2, bei der das oder die Gegenion(en) für mindestens einen Teil der Carboxylgruppen in der vernetzten Acrylatfaser ein oder mehrere Magnesium- und/oder Zinkion(en) ist/sind.

4. Vernetzte Acrylatfaser nach Anspruch 3, wobei das Gegenion für mindestens einen Teil der Carboxylgruppen in der vernetzten Acrylatfaser ein Magnesiumion ist, der LOI-Wert (Limiting Oxygen Index) 30 bis 50 beträgt und die Aufnahmerate zur Feuchtigkeitssättigung 20 bis 60 Gewichts-% beträgt.

5. Verfahren zur Herstellung einer vernetzten Acrylatfaser, **dadurch gekennzeichnet, dass** die Behandlungen (a) Behandlung zum Einbringen einer Vernetzung mit einer Hydrazinverbindung, (b) Behandlung mit einem Peroxid und (c) Hydrolysebehandlung mit einer Alkalimetallverbindung an einer Acrylnitritfaser in der Abfolge (a), (b) und (c) vorgenommen werden.

6. Verfahren zur Herstellung einer vernetzten Acrylatfaser, **dadurch gekennzeichnet, dass** die Behandlungen (a) Behandlung zum Einbringen einer Vernetzung mit einer Hydrazinverbindung, (b) Behandlung mit einem Peroxid und (c) Hydrolysebehandlung mit einer Alkalimetallverbindung an einer Acrylnitrilfaser in einer Abfolge derart vorgenommen werden, dass nachdem (a) erfolgt ist, (b) und (c) dann gemeinsam vorgenommen werden.

## Revendications

1. Fibre d'acrylate réticulée ayant une couleur dont L* a une valeur de 60 à 75, a* a une valeur de 5,0 à 14,5 et b* a une valeur de 23,0 à 30,0 suivant la méthode d'expression stipulée par JIS-Z-8729.

2. Fibre d'acrylate réticulée suivant la revendication 1, dans laquelle les traitements comprenant (a) un traitement pour l'introduction d'une réticulation par un dérivé d'hydrazine, (b) un traitement par un peroxyde et (c) un traitement d'hydrolyse utilisant un composé de métal alcalin sont appliqués à une fibre d'acrylonitrile dans l'ordre (a), (b) et (c) ou dans un ordre tel que, après application de (a), (b) et (c) soient ensuite appliqués ensemble.

3. Fibre d'acrylate réticulée suivant la revendication 1 ou 2, dans laquelle le ou les ions complémentaires pour au moins une partie des groupes carboxyle dans la fibre d'acrylate réticulée est/sont un/des ion(s) magnésium et/ou zinc.

4. Fibre d'acrylate réticulée suivant la revendication 3, dans laquelle l'ion complémentaire pour au moins une partie des groupes carboxyle dans la fibre d'acrylate réticulée est l'ion magnésium, l'indice limite d'oxygène va de 30 à 50 et la vitesse d'absorption d'humidité à saturation va de 20 à 60 % en poids.

5. Procédé pour la production d'une fibre d'acrylate réticulée, **caractérisé en ce que** les traitements comprenant (a) un traitement pour l'introduction d'une réticulation par un dérivé d'hydrazine, (b) un traitement par un peroxyde et (c) un traitement d'hydrolyse utilisant un composé de métal alcalin sont appliqués à une fibre d'acrylonitrile dans l'ordre (a), (b) et (c).

6. Procédé pour la production d'une fibre d'acrylate réticulée, **caractérisé en ce que** les traitements comprenant (a) un traitement pour l'introduction d'une réticulation par un dérivé d'hydrazine, (b) un traitement par un peroxyde et (c) un traitement d'hydrolyse utilisant un composé de métal alcalin sont appliqués à une fibre d'acrylonitrile dans un ordre tel que, après application de (a), (b) et (c) soient ensuite appliqués ensemble.
